

## UNITED STATES PATENT OFFICE.

HERMANN SCHMIDT, OF WIESDORF-ON-THE-RHINE, AND EMIL HUBERT, OF ELBERFELD, GERMANY, ASSIGNORS TO I. G. FARBNINDUSTRIE AKTIENGESELLSCHAFT, OF FRANKFORT-ON-THE-MAIN, GERMANY.

## METHOD OF SPINNING ARTIFICIAL SILK.

No Drawing. Application filed April 4, 1927, Serial No. 180,994, and in Germany June 11, 1926.

This invention relates to a new method of spinning artificial silk from cuprammonium cellulose solutions and involves the use of an aqueous precipitating bath containing dissolved carbon dioxide or carbonic acid or its chemical equivalent, a soluble bicarbonate. The invention is particularly applicable in the so-called stretch-spinning process.

Heretofore it has been regarded as being important in the spinning of artificial silk to use a de-aerated precipitating bath, i. e., a bath which is free or has been freed of dissolved gases.

It has now been found that considerably improved results may be obtained, if the precipitating bath used in the spinning of artificial silk from cuprammonium cellulose solutions is not de-aerated, but on the contrary contains dissolved carbon dioxide or bicarbonate. The use of such a precipitating bath gives silk of greater tensile strength and elasticity than silk produced by spinning into customary de-aerated bath and besides the use of a carbon dioxide containing bath prevents, to a large extent, the deposition of copper salts upon the spinning nozzle. Dissolved carbon dioxide or carbonic acid and soluble bicarbonates have entirely similar effects, but the use of bicarbonates has the advantage that the carbon dioxide component is not expelled by raising the temperature of the precipitating bath, i. e., the bath may be used at ordinary or somewhat elevated temperatures, if desired, without loss of the effective carbon dioxide. Any soluble bicarbonate such as the alkali metal and alkaline earth metal bicarbonates, e. g., sodium bicarbonate or calcium bicarbonate may be employed. It will be understood the aqueous precipitating bath may contain carbon dioxide dissolved therein and chemically combined with water as the hypothetical acid  $H_2CO_3$ , or chemically combined with metals as bi- or acid carbonates as  $NaHCO_3$ . The bicarbonate may be added to the bath as such, for instance, as sodium bicarbonate or formed in the bath by treating a solution of a metal hydroxide or carbonate with carbon dioxide.

It will be further understood that in the

appended claims where reference is made to dissolved carbon dioxide, carbonic acid and acid carbonates are embraced.

The following examples illustrate the invention:

*Example 1.*—Cuprammonium cellulose solution is precipitated according to the stretch spinning process in a spinning vessel of the customary type with water at about 32° C. containing approximately 10 to 20 mg. of free carbonic acid per liter. It is likewise possible in this spinning process to employ water possessing slight hardness. The further treatment of the precipitated threads is then effected according to the customary methods.

*Example 2.*—Cuprammonium cellulose solution is precipitated in water containing approximately 2 grams of sodium bicarbonate per liter in a spinning vessel, for example according to the process of German Pat. No. 220,051. The further treatment of the precipitated threads is effected according to the customary methods.

## Claims:

1. Process for the manufacture of artificial silk from a cuprammonium cellulose solution which comprises spinning the solution into an aqueous precipitating bath containing dissolved carbon dioxide.

2. Process for the manufacture of artificial silk from a cuprammonium cellulose solution according to the stretch-spinning method which comprises spinning the solution into an aqueous precipitating bath containing dissolved carbon dioxide.

3. Process for the manufacture of artificial silk which comprises spinning a cuprammonium cellulose solution into an aqueous precipitating bath containing a bicarbonate in solution.

4. Process for the manufacture of artificial silk which comprises spinning a cuprammonium cellulose solution into an aqueous precipitating bath containing a bicarbonate of an alkali forming metal in solution.

In testimony whereof we have hereunto set our hands.

HERMANN SCHMIDT.  
EMIL HUBERT.